

## UNITED STATES PATENT OFFICE

2,357,211

## SULPHURIZED OILS

Bert H. Lincoln and Waldo L. Steiner, Ponca City,  
Oklahoma, assignors to Continental Oil Company,  
Ponca City, Okla., a corporation of Delaware

No Drawing. Application January 4, 1940,  
Serial No. 312,408

2 Claims. (Cl. 252—48)

This invention relates to sulphurized oils and new compositions of matter used in the preparation thereof and is a continuation-in-part of our co-pending application, Serial No. 257,458, filed February 20, 1939, issued January 4, 1940, as Patent No. 2,186,646.

It has long been known that sulphur compounds, when added to lubricating oils, impart certain properties to the mixtures which are of great value when these mixtures are used as lubricants for very heavy duty such as is encountered in the lubrication of automotive gears of the hypoid and spiral bevel types and other power transmission gears and for the lubrication of cutting tools such as are used in cutting and threading steel pipe. The exact manner in which the sulphur compounds, with respect to the cutting lubricants, act to produce these results is not known with any degree of certainty. It is more than a matter of the increased film strength which sulphur compounds impart to lubricating oils, since, for each sulphur compound that may be added to a lubricating oil to increase its film strength, there is an optimum percentage above which there is no tendency to obtain further increase with greater percentages of the sulphur compound. On the other hand, there seems to be no limit to the improvement of a cutting oil that can be obtained by increasing its sulphur content, at least as far as the smoothness of the metal cut obtained with it is concerned.

All sulphur compounds do not have this beneficial effect on lubricants to the same degree for the same amount of sulphur, as will be brought out in the examples given hereinbelow; and to most of those now in use, there are certain definite objections. The most common sulphur compounds used for blending with lubricating oils are the sulphuretted glycerides of the unsaturated fatty acids. These usually contain about 12 per cent sulphur. Sulphuretted lard oil is a typical example. These compounds are not entirely satisfactory for blending purposes for several reasons. The sulphuretted glycerides are very viscous and hard to handle and raise the pour point of the oil with which they are blended, have a very strong odor of hydrogen sulphide, are irritating to the skin of the operators working with them, are not as stable as desired when in use and do not give a good cut when used in a cutting lubricant, do not give a very high film strength when used in an extreme pressure lubricant, are not entirely oil soluble, and are not refinable to any extent.

Even with using a large percentage of these

sulphur-base oils, cutting lubricants are obtained which are rather inefficient as far as cutting qualities are concerned, objectionable on account of odor, irritating to the skin of the operator and 5 in case of slight cuts on the hand cause sores difficult to heal, are very viscous when cold, are not stable to high temperatures while in use, and break down and release H<sub>2</sub>S.

An extreme pressure lubricant for gears which 10 is made from the conventional sulphuretted glycerides, such as lard oil, has many defects. In the first place, this type of sulphur-base blend is not as stable as is desired to the copper strip corrosion test, which some automobile manufacturers now require for sulphur-base lubricants. Secondly, the film strength is not very high; and last, the pour point of the lubricant is raised five degrees to 25 degrees F., depending upon the type of petroleum base oil used.

20 We have discovered that the sulphuretted or sulphurized synthetic monohydric and dihydric alcohol esters of organic acids make excellent sulphur bases for blending with lubricants for preparing superior cutting oils and gear lubricants. By the term "sulphurize" we mean the 25 introduction of sulphur in the form in which it is introduced into a synthetic ester by means of sulphur or a halide of sulphur. These compounds are superior to the conventional sulphuretted 30 glycerides of unsaturated fatty acids in a number of ways. To begin with, they are in general much less viscous even when containing a much larger percentage of sulphur and are therefore easier to handle. They may be easily and 35 permanently freed from the odor of hydrogen sulphide by blowing for a few minutes with sulphur dioxide after sulphuretting, followed by an inert gas such as carbon dioxide. They are, as a group, much more stable to heat than the sulphuretted 40 glycerides and consequently do not break down and release H<sub>2</sub>S in service as readily. When the glyceride breaks down, glycerine is released which forms gum and is generally objectionable.

When used in a cutting oil, they do not irritate 45 the skin of the operators. They are cheaper because about twice as much sulphur may be added to this type of compound as can be added to the glycerides, and thus they give a more concentrated base. Another important advantage 50 of these sulphuretted or sulphurized synthetic monohydric and dihydric alcohol esters is that they are more soluble in petroleum lubricants than their corresponding sulphuretted glycerides. The latter have a marked tendency to show a sludge-like deposit on the bottom of the con-

tainer in which a blend of this type base and a petroleum lubricant has stood for some time. The reason for this phenomenon is that glycerides tend to polymerize on sulphuretting and form oil insoluble polymers, whereas their corresponding synthetic monohydric esters show little or no tendency to polymerize on sulphuretting or sulphurizing. The pour point of blends made with a petroleum lubricant is higher by 10° to 25° F. (depending on the type of lubricant) when a sulphuretted glyceride is used than when the corresponding sulphuretted or sulphurized synthetic monohydric alcohol ester is used. The latter do not affect the emulsion characteristics and decrease the sludge-forming tendencies of the base oil with which they are blended. The sulphuretted glycerides cause emulsion trouble and increase sludge formation.

The viscosity of the sulphuretted glyceride blends is very much higher for the same amount of added sulphur at temperatures from 0 degrees to 50 degrees F. than similar blends where the sulphuretted or sulphurized synthetic monohydric alcohol esters of the same acids are used. This is a very important factor when considering either a cutting oil or a power transmission gear lubricant. In the case of the former, it is frequently difficult to obtain a good flow of the cutting oil from the sump of the machines on cold mornings in a shop that is not too well heated. Under these conditions, the machines do poor work; and the cutting tools are dulled. The disadvantages of a high pour test and high viscosity at cold weather temperatures in the case of gear lubricants cause excess loss of power in overcoming the internal friction of the lubricant and difficulty in shifting of gears in the case of automobile transmission gears.

We have found more particularly that certain synthetic esters of mono and dihydric phenols with organic acids are especially suited to sulphurization and use when blended in mineral oils for lubricating purposes. The mono and dihydric phenols which we may use may be mono- or bi- or polycyclic and may contain various substituents and/or side chains in addition to the one or two hydroxyl groups. The organic acids which we may use to esterify with such phenols are of various types, including the acids (free or combined) occurring in natural fats, waxes, and saponifiable oils, as well as synthetic acids. Of these acids, however, we prefer the unsaturated ones because their esters are easier to sulphurize than the saturated ones. The latter may be satisfactorily used if higher temperatures and longer times of sulphurizing are employed as described below.

Some examples of the esters we may sulphurize are given below, and it is to be understood that any of the phenolic components mentioned may be combined with any of the acid radicals mentioned to obtain further examples of the esters we may sulphurize. It is also to be understood that the following esters, when sulphurized and blended with mineral oil, are to be considered as examples of our invention:

Phenyl cinnamate  
Phenol esters of corn oil acids

Phenyl mellitate

Hydroquinone distearate

Resorcinol esters (di) of soy bean oil acids

Catechol esters (di) of wool fat acids

Phenyl oleate

*a*-Naphthyl linoleate

*b*-Naphthyl linoleate

Ester of 8-hydroxyquinoline with beeswax acids  
Phenyl esters of sperm oil acids

Anthryl oleate

Cresyl abietate

5 Phenolic esters of the acids of naturally occurring waxes such as carnauba, candelilla, gondang, Japan, montan, and bayberry waxes  
Phenyl linoleate.

10 Naturally occurring oils and waxes as such containing monohydric alcohol esters of organic acids have proved unsatisfactory for use in this invention. The reason for this appears to be that these naturally occurring substances are a mixture of esters with naturally occurring impurities such as glycerides, high molecular weight alcohols, hydrocarbons, often nitrogen compounds, and other impurities. Some of the oils and waxes in this group are sperm oil and similar whale oils, wool fat or wool grease, beeswax, carnauba wax, and candelilla wax. Sperm oil contains from 5 per cent to 25 per cent of glyceride, which makes it unsatisfactory. It also contains an appreciable amount of free high molecular weight alcohols which are objectionable, since they also give relatively unstable derivatives on sulfurizing. The removal of the monohydric or dihydric alcohol esters as such from the glycerides, free alcohol, and other impurities in the naturally occurring material is not commercially feasible.

20 When sperm oil is sulphurized, a product is obtained which does not lend itself to refining as do the sulphurized relatively pure synthetic esters; consequently it cannot be used in a crankcase lubricant as an oiliness and film strength improver or as a sludge inhibitor because of its adverse effect on color, emulsibility, and cloud test. The objectionable characteristics of the glycerides as described previously are in general also pertinent to the sulphurized naturally occurring esters with only a few exceptions.

25 Wool fat or wool grease contains monohydric alcohol esters but is not satisfactory for use in our invention because of naturally occurring impurities found therein. These consist of alkali salts of fatty acids and free high molecular weight alcohols which yield relatively unstable sulphur derivatives. Sulphurized wool fat is not a satisfactory lubricating oil addition agent because it is not stable enough to allow refining; and when added to mineral oils, the resultant blend will not give a satisfactory emulsion or cloud test. Sulphurized wool fat darkens the color of the oil. It also breaks down at relatively low temperatures (compared with sulphurized synthetic esters) and releases H<sub>2</sub>S, which is objectionable. Hence wool fat would not give a satisfactory lubricating oil addition agent after sulphurizing.

30 Beeswax contains 10 to 20 per cent free fatty acid and 10 to 15 per cent hydrocarbons and is therefore unsuited for the production of a sulphurized addition agent for lubricating oils.

Candelilla wax contains, besides monohydric alcohol esters, about 10 per cent or more free fatty acid and about 50 per cent hydrocarbons. Carnauba wax contains some monohydric alcohol esters, but these are mixed with a complex variety of impurities such as free fatty acids, hydrocarbons, and free high molecular weight alcohols; and therefore neither candelilla nor carnauba wax is suitable for use as lubricating oil addition agents after being sulphurized.

35 However, the above-mentioned materials, namely naturally occurring wax containing saponifiable oils, sperm oil and similar whale oils,

wool fat, wool grease, beeswax, carnauba wax, and candelilla wax do contain considerable quantities of high molecular weight acids (free and combined) which are suitable for use in our invention after saponification and separation of the acids and esterification with a mono- or dihydric phenol. This renders usable the valuable acids of the naturally occurring waxes and wax-containing saponifiable oils. We believe this is largely due to the decomposition of glycerides and removal of the glycerol present in some of these materials, but we do not wish to be bound by this supposition but only by the appended claims interpreted as broadly as the prior art permits.

The sulphurization of our phenolic esters may be accomplished by heating the synthetic ester with sulphur or a halide of sulphur in the presence or absence of a solvent. The temperature used depends on the particular synthetic ester. About 350 to 380° F. is used on esters derived from unsaturated acids and about 380 to 450° F. is necessary for esters derived from saturated acids. As solvents, petroleum fractions having initial boiling points of 350° F. and higher may be used up to such light lubricating oils as a neutral oil having a viscosity of 150 S. S. U. at 100° F. The more volatile solvents of this type may be removed by distillation with steam or in a vacuum while the higher boiling neutral oils may be left in the sulphurized ester if they are taken into consideration when subsequent blends are made.

In sulphurizing our phenolic esters we may use elemental sulphur or various compounds of sulphur including sulphur monochloride, sulphur dichloride, phosphorus pentasulphide, phosphorus trisulphide, polysulphides, and the like. Each of these reagents gives somewhat different products. Furthermore, by variations in the conditions of sulphurization, we may obtain two general types of products from each reagent regardless of sulphur content. One of these contains some active sulphur, and the other contains no active sulphur; that is, all the sulphur is in an inactive form. By active sulphur we mean that form which is present when a blend of the sulphurized material in 150 neutral oil containing one per cent of added sulphur will appreciably discolor a bright copper strip immersed therein and held at 210° F. for 30 minutes. If the copper strip is not appreciably discolored, all the sulphur present is in an inactive form.

Both types of sulphurized products are useful for different purposes. For example, materials containing active sulphur are more effective components of gear lubricants and the like where extreme pressure is used and no easily corrodible metals are present. For crankcase use, however, especially where bearing metals sensitive to corrosion are employed, our product containing only inactive sulphur is preferred.

Various factors must be considered in the preparation of our sulphurized phenolic esters containing active and inactive sulphur:

**1. Reagent.**—In general for the preparation of sulphurized phenolic esters containing active sulphur, we prefer to use elemental sulphur combined with short times of heating and lower temperatures. The sulphur compounds such as chlorides of sulphur and sulphides of phosphorus are more likely to give products containing only inactive sulphur and are not so flexible with regard to variations in other conditions as sulphur itself; however it is possible to use sulphur

compounds to obtain products with active sulphur.

**2. Proportions of reagents.**—For the preparation of products with active sulphur, we prefer to use large proportions of sulphur or sulphur compounds because it is easier to obtain the desired product, other factors being constant. It is possible, however, at lower temperature and with shorter periods of heating especially in solvents, to obtain active sulphur containing products using small amounts of sulphur. By controlling reagents and conditions we are able to obtain sulphur bearing derivatives with 2 to 20 per cent or more sulphur. For any given sulphur content, we may obtain products containing active sulphur or containing only inactive sulphur.

3. *Temperature*.—Higher temperatures tend to fix the sulphur in inactive combination and are used when a stable sulphurized synthetic ester is desired. Use of lower temperatures with the same reagents and otherwise the same conditions gives products containing active sulphur which are especially useful for cutting oils and extreme pressure gear lubricants when blended with hydrocarbon oils and other ingredients.

4. *Time*.—We heat our reactants for a relatively short time to produce materials with active sulphur and for a relatively long time to obtain only inactive sulphur in our products. A short time at a high temperature may be selected which is the equivalent of a longer time at a lower temperature within certain limits. There is, however, a most suitable range of temperature below which the time required is unreasonably long.

5. *Solvents.*—Insert solvents may be employed; and, in general, they have the effect of limiting the highest temperature used in a particular sulphurization. If the solvent does not dissolve the sulphur or sulphur compound appreciably, the rate of reaction is slower and the formation of products containing active sulphur is favored. If the solvent dissolves the sulphur or sulphur compound, the reaction proceeds more rapidly; and products containing only inactive sulphur are more readily obtained.

6. Unrefined products are more likely to contain active sulphur than unrefined products.

We vary the quantities of refining reagents, for example, sulphuric acid and clay, and also their concentration, time, and temperature of contact, etc., to obtain thorough refining when a very stable product is desired. The refining may be milder or even omitted when an active sulphur product is sought.

7. *Pressure.*—Under superatmospheric pressure the sulphur is more stably fixed in the same time and under the otherwise same conditions, and this is a useful modification of our process in order to obtain products containing only inactive sulphur.

While there is no specific limitation to the amount of added sulphur in the form of sulphurized phenolic esters that should be used in preparing different lubricants, usually 1 to 4 per cent or more may be used for cutting oils; and about .5 to 2.5 per cent or more will usually be sufficient for gear and other extreme pressure lubricants. As little as .001 per cent or a little less and up to .25 per cent or more may be used in oils for use in automobile crankcases.

The above ratios of sulphur to the petroleum base oil for its different uses are not intended to limit the scope of this invention, since smaller

or larger quantities may be used in any case with results which are partially satisfactory. They are given because generally speaking the optimum results can be obtained by using the ratios within the limits that are suggested.

The hydrocarbon oils which are used in blending with the sulphurized phenolic esters are not limited to the hydrocarbon oils cited in the examples but are to include any oil of any type or viscosity such as may be required by the lubricant in question. These different types of oils may be unrefined mineral oil or oil refined by any method, such as by the use of acids, alkalis, or solvents, or any combination of said refining processes. Other types are synthetic oils made by polymerization or similar processes and hydrogenated oils.

Sulphur dioxide and carbon dioxide have been mentioned as agents for blowing sulphurized synthetic esters and it is to be understood that

the inventors are in no way limited to any particular refining process and that other gaseous or liquid refining agents as nitrogen or alkali solutions and acid solutions may be used in refining sulphurized phenolic esters of certain character and for certain purposes.

Having thus described our invention, we claim:

1. A lubricant comprising in combination a major amount of a lubricating oil and a minor amount of a sulphurized ester of phenol and an unsaturated organic acid, said ester being sulphurized by a compound containing phosphorus and sulphur.

2. A lubricant comprising in combination a major amount of a lubricating oil and a minor amount of a sulphurized ester of phenol and an unsaturated organic acid, said ester being sulphurized by phosphorus pentasulphide.

BERT H. LINCOLN.

WALDO L. STEINER.